

Dec. 16, 1930.

N. C. BEIM

1,784,809

LUBRICANT AND PROCESS OF PRODUCING THE SAME

Filed March 19, 1928



INVENTOR.

Nels C. Beim,  
BY Bryan B. Collings  
ATTORNEY.

## UNITED STATES PATENT OFFICE

NELS C. BEIM, OF MINNEAPOLIS, MINNESOTA

## LUBRICANT AND PROCESS OF PRODUCING THE SAME

Application filed March 19, 1928. Serial No. 262,959.

This invention relates to the production of an improved lubricant, and more particularly to a lubricating oil especially adapted for use in internal combustion engines and similar motors, and has for one of its objects to provide an improved lubricant which will be more efficient in use than those which have been heretofore proposed.

A further object of the invention is to produce a lubricating oil possessing an inherent complete laminar orientation of the lubricating structure, resulting in such a high concentration of true lubricating value as to make possible the use of a single viscosity or weight of the product for all internal combustion engine lubricating requirements; or in other words, one grade of oil for all motors.

A further object of the invention is the stripping or elimination of the more volatile, non-working, superfluous, fractions resulting in greater resistance to heat and pressure, as an additional aid toward the practicability of the use of one supergrade for all motors.

A still further object of the invention is to provide an improved process for the manufacture of the above described lubricant.

With the above and other objects in view, which will appear as the description proceeds, the invention consists in the novel combinations of ingredients constituting the improved lubricant, and in the novel steps and combinations of steps constituting the process, all as will appear more fully below, and be particularly pointed out in the claim.

In order that the precise nature of the invention may be better understood, it may be said that it is well known at present that the various makes of internal combustion engines possess different characteristics which indicate the use of many different grades of lubricating oils in order to attain the highest efficiency; and that of the oils now in common use, any one grade which may produce the proper lubrication and greatest efficiency in any particular type or make of motor, may be wholly unsuited for a different make. It is well recognized in the industry that it is highly desirable to provide a lubricating medium suitable to all motors indiscriminately,

and the medium hereinafter described has been found to attain this desirable result.

In the preparation of this lubricant, substantially equal quantities of lubricating components consisting of viscous stripped neutral, (300 sec. at 100° F.) 120-130 viscosity at 210° F. and bright stock, paraffine base, are each injected into a closed devolatilizing chamber through one-quarter inch nozzles under pressure of approximately two hundred pounds, with additional turbulence being set up in a chamber by means of suitably placed baffle plates in the direct line of the injection spray; this contrivance resulting in a complete and intimate intermixture both physical and structural.

Thereafter, this mixture is subject to a temperature of 425° F. for thirty minutes, through the use of superheated steam coils, and about 15% of the mixture in the aforementioned chamber, distilled off with the additional aid of a partial vacuum. (10# to square inch.) Then to this residuum remaining in the chamber, is introduced .3 of 1% of magnesium stearate, rich in colloids, which is thoroughly intermixed by agitation with air.

The resultant product is then finished filtered through infusorial earth, to the desired color.

The above treatment is found to produce a lubricant in which the colloidal hydrocarbons are so concentrated as to permit of the use of a single grade of the lubricant in any motor.

In the accompanying drawing forming a part of this specification, the figure is a more or less diagrammatic sectional view of one form of apparatus which may be employed in carrying out the present process. In the said drawing, 1 indicates a closed chamber of suitable construction, provided with a series of staggered baffles 2, which may support steam pipes 3. These said pipes, however, may be arranged and supported in any other appropriate manner. Nozzles 4 and 4' are provided through which the lubricating components may be introduced into the chamber 1 under pressure in converging streams or sprays, and the chamber is also provided with a draw-off pipe 5, controlled

by a valve 6, and an outlet conduit 7, controlled by a valve 8, which conduit 7 may be connected to a suitable vacuum pump (not shown) for reducing the pressures within the chamber at certain stages, all as previously set forth. The stearate and the agitating air may be introduced through the pipes 10 having the control valves 11.

It is obvious that those skilled in the art may vary the precise temperatures, times, and pressures employed within certain limits, as well as other minor details of the process, without departing from the spirit of the invention, and, therefore, it is not wished to be limited to the above disclosure except as may be required by the claim.

What is claimed is:

The process of producing a lubricant for internal combustion motors and the like, which consists in injecting substantially equal quantities of two grades of commercial lubricating oil into a closed chamber under heavy pressure, whereby a substantially complete physical and structural intermixture of the two results; subjecting the mixture to the action of a partial vacuum of approximately 10 lbs.; heating the mixture to approximately 425° F. to drive off a portion of the lighter fractions; adding approximately .3 of 1% of magnesium stearate to the residuum while agitating the mixture; and filtering the resulting product.

In testimony whereof I affix my signature.  
NELS C. BEIM.

35

40

45

50

55

60

65